

1

3,287,894

**METHOD OF PREPARING RAYON TYING TWINE**  
 Richard MacHenry, Prospect Park, Pa., assignor to FMC Corporation, Philadelphia, Pa., a corporation of Delaware

No Drawing. Filed June 25, 1964, Ser. No. 378,063  
 4 Claims. (Cl. 57—164)

This invention relates to a method of preparing rayon tying twine. More particularly, it relates to a method of preparing rayon tying twine in a package.

The machine application and tying of twine such as found in "tag" machines for stringing price tags and labels, requires a twine which will not shell off of its cone or ravel, which will tie a suitable knot, and perform satisfactorily on the machine itself.

Rayon yarn would be desirable for use as a twine since it is relatively inexpensive and strong. Rayon alone, even when the strands are twisted, has not been found suitable as a twine for machine operation. Several finishes and coatings have been applied without complete success.

It is an object of this invention to provide a method for the preparation of a suitable tying twine package for machine application and tying.

This and other objects are met in accordance with this invention wherein the method of preparing rayon tying twine comprises twisting rayon yarn from 2 to 6 turns per inch, treating said yarn with a homogeneous mixture of from 90 to 95%, based on the volume of the mixture, of a C<sub>1</sub>—C<sub>4</sub> alkanol and an aqueous dispersion of polyvinyl acetate at a solids concentration of from about 25 to about 65%, preferably about 30 to 40% by weight, winding the wet yarn into a package, and drying the package.

The twisting of the yarn is necessary to obtain a rayon twine having a reduced tendency to ravel. While 2 to 6 turns per inch are required about 4 to 5 turns per inch are preferred.

The alkanols for this invention are those which are miscible with aqueous mediums and include, e.g., methanol, ethanol, n-propanol, isopropanol, and t-butanol. Isopropanol is preferred based on expense. The alkanols, aside from being miscible with water, are substantially non-toxic, do not degrade or swell cellulose material and have a sufficiently high vapor pressure to evaporate from the yarn in a reasonably short time. The use of the alkanol as the carrier is responsible for producing a non-shelling, firm package as compared to one produced with a water diluted polyvinyl acetate emulsion.

Emulsions of polyvinyl acetate resins are generally supplied at a high solids concentration and may be diluted with water to obtain the desired consistency. After diluting, the emulsion is mixed with the alkanol to obtain the prescribed composition.

Additive materials in small amounts may be added to the composition including plasticizers, pigments, coales-

2

ing agents and surface modifying agents such as clays and waxes.

The following example is set forth to demonstrate the method of this invention.

*Example*

4000 ccs. of a polyvinyl acetate emulsion supplied at a solids concentration of about 55% was mixed with 4000 ccs. of water and stirred until well distributed.

10 8000 ccs. of the diluted emulsion was added to 34 gallons of isopropanol and stirred to obtain a homogeneous mixture.

15 This mixture was applied to rayon yarn of 1780 denier having 4.5 turns per inch and the excess mixture stripped off. The yarn was then coned wet and the cone permitted to dry.

20 This cone was a non-shelling, non-ravelling twine which formed a satisfactory knot on a tag machine. The finished rayon twine is stronger and less expensive than comparable cotton string.

25 Various changes and modifications may be made practicing the invention without departing from the spirit and scope thereof and, therefore, the invention is not to be limited except as defined in the appended claims.

I claim:

1. A method of preparing rayon tying twine which comprises twisting rayon yarn from 2 to 6 turns per inch, treating said yarn with a homogeneous mixture of from 90 to 95%, based on the volume of the mixture of a C<sub>1</sub>—C<sub>4</sub> alkanol and an aqueous dispersion of polyvinyl acetate at a solids concentration of from 25 to 65% based on the weight of the dispersion, winding the wet yarn into a package, and drying the package.

2. The method of claim 1 wherein the alkanol is isopropanol.

3. The method of claim 2 wherein the dispersion of polyvinyl acetate has a solids concentration of 30 to 40%.

4. A method of preparing rayon tying twine which comprises twisting rayon yarn from 4 to 5 turns per inch, treating said yarn with a homogeneous mixture of about 94%, based on the volume of the mixture, of isopropanol and an aqueous dispersion of polyvinyl acetate at a solids concentration of from 30 to 40% based on the weight of the dispersion, winding the wet yarn to a package, and drying the package.

**References Cited by the Examiner**

**UNITED STATES PATENTS**

- |    |           |         |               |          |
|----|-----------|---------|---------------|----------|
| 50 | 2,775,860 | 1/1957  | Morrison      | 57—164 X |
|    | 2,856,750 | 10/1958 | Lewis         | 57—153   |
|    | 2,964,262 | 12/1960 | Lessig et al. | 57—164 X |

FRANK J. COHEN, Primary Examiner.

55 J. PETRAKES, Assistant Examiner.